

June 15, 1926.

1,588,429

A. J. WACHSMUTH

METHOD OF MAKING ARTIFICIAL CANE

Filed June 13, 1921



Fig. 1.



Fig. 2.



Fig. 3.



Fig. 4.



Fig. 5.



Fig. 6.

Inventor

Albert J. Wachsmuth

By Frank E. Liverance, Jr.  
Attorney.

Patented June 15, 1926.

1,588,429

# UNITED STATES PATENT OFFICE.

ALBERT J. WACHSMUTH, OF MUSKEGON, MICHIGAN.

## METHOD OF MAKING ARTIFICIAL CANE.

Application filed June 13, 1921. Serial No. 476,984.

This invention relates to a method or process of making artificial cane from paper. It is a primary object of the present invention to use paper and fold it into a compact length, a plurality of longitudinal folds of the paper being made, the paper previous to such folding being coated with glue or other cementitious material so that when folded, the different contacting surfaces of the paper adhere to each other, thereby making a firm strip or length of cane, and also having possibilities for forming into different shapes by running the same through suitable forming and compressing rollers to shape the cane to desired form. In practice, I use two strips or lengths of paper in making the artificial cane, coating the same with the cementitious material and then folding them lengthwise a number of times. The invention, however, is not limited in the use of any specified number of strips, but comprehends the method outlined, irrespective of the number of strips of paper used or the exact number of longitudinal folds made.

For an understanding of the invention, reference may be had to the following description, taken in connection with the accompanying drawing, in which,

Fig. 1 is a perspective view illustrating the sequence of the foldings made in the strips of paper used for the production of the cane.

Figs. 2, 3, 4 and 5, are sections taken transversely on the planes of lines 2—2, 3—3, 4—4 and 5—5, respectively of Fig. 1, and

Fig. 6 is an enlarged transverse section showing the cane made pressed or rolled to a finished more or less oval form.

Like reference characters refer to like parts in the different figures of the drawing.

In the carrying out of the process or method, two strips of paper 1 and 2 are used, preferably, and brought together one over the other, being coated with glue or similar cementing material before being brought together so that the same adhere when in contact. The next step of the process is to fold the two strips between their edges longitudinally, as indicated at 3, the outer strip being folded to make two sides 4 and 5, and the inner strip two sides 6 and 7, the sides 4 and 6 being wider than sides 5 and 7, as shown in Fig. 3. This makes four thicknesses of paper cemented together. The next step is to again fold the four thicknesses longitudinally between their edges as indicated at 8, making eight thick-

nesses of the paper cemented together, as indicated in Fig. 4. As a final step the eight thicknesses of paper are again folded longitudinally between their edges, as indicated at 9, the resulting form being substantially rectangular in cross section and having practically fourteen thicknesses of the paper cemented together, as shown in Fig. 5, the shortening of the sides 5 and 7 in the first instance coupled with the successive foldings practically eliminating two thicknesses of the paper in the final fold as shown. It is to be understood that the thickness of the paper is necessarily exaggerated in the drawing and the proportions are not exact but are sufficiently so to illustrate the steps of the process. The final form, shown enlarged in Fig. 5 is one that is readily rolled or pressed into the half-oval form indicated in enlarged section in Fig. 6, and as a final culminating step of the process the folded cemented length of paper is pressed or rolled to such form, preferably, making a smooth, tough and substantial artificial cane capable of use in practically all places where the natural cane is used.

It is evident that different sizes of the cane may be used and that larger sizes may be made by merely using wider strips of paper 1 and 2 in the first instance. It is also very evident that, so far as the process is concerned, the strips 1 and 2 need not be separated, as a single strip of a width equal to the combined widths of the two strips and folded centrally and longitudinally would have the same effect as two separated strips. Accordingly, I do not limit myself to the exact disclosure as comprehending the process which I have devised, but consider the same to comprehend the various equivalent steps which I have mentioned, as well as others not specifically stated but which will occur to others.

The process described is practical and has been followed successfully in actual practice. The cane made is flexible, tough and durable, easily worked to a desired shape or form, and practical for use in every way.

I claim:

1. The herein described process of making artificial cane or the like, which consists in coating a strip of paper with cementing material and thereafter folding and refolding the strip longitudinally between its edges to make a plurality of overlying laminations of paper, substantially as described.

2. The herein described process of making artificial cane or the like, which consists in coating a plurality of elongated strips of paper with cementing material, bringing said strips together, and thereafter folding and refolding the strips a plurality of times longitudinally between the edges thereof to make a plurality of overlying laminations of paper.
- 10 3. The herein described process of making artificial cane or the like, which consists in longitudinally folding and refolding an elongated strip of paper a plurality of times between its edges to make a plurality of overlying laminations of paper and cementing the same together.
4. The herein described process of making artificial cane or the like, which consists in superimposing a plurality of elongated strips of paper, then longitudinally folding and refolding said strips a plurality of times between their edges to make a plurality of overlying laminations of paper and cementing the folds together, substantially as described.

In testimony whereof I affix my signature.

ALBERT J. WACHSMUTH.